

## UNITED STATES PATENT OFFICE

FRITS ELLINGER, OF THE HAGUE, NETHERLANDS, ASSIGNOR TO MIJNBOUW EN  
HANDELSMAATSCHAPPIJ, "WONOH GEDEH," OF THE HAGUE, NETHERLANDS

## PROCESS FOR LIBERATING IODINE IN IODINE-CONTAINING MINERAL WATERS

No Drawing. Application filed March 7, 1929, Serial No. 345,229, and in the Netherlands March 10, 1928.

For obtaining iodine several methods are already known, including obtaining iodine and iodine compounds from iodine-containing charcoal.

5 The present invention relates to a process for liberating iodine from its compounds in iodine-containing mineral waters, whilst the liberated iodine can then be adsorbed by charcoal.

10 It is known that many oxidizing agents are suitable for liberating iodine from iodides. In Abegg's Handbuch der Anorg. Chemie Vol. IV, 2 (1913) page 348 it is stated that permanganic acid is specially suitable

15 for separating iodine from iodides in order to obtain a particularly pure iodine.

This method has however never found commercial application, nor has it ever been proposed for liberating iodine from iodine-containing mineral spring-waters, in which only very small quantities of iodides besides a large excess of other salts are present.

20 Until now, for liberating iodine from spring-waters only sodium nitrite in acid solution or nitric sulphuric acid has been used. These chemicals have been considered the most suitable for the object on account of their cheapness and it has never been proposed to use anything else. It has now been

25 found, however, that the use of nitrite as an oxidizing agent is not profitable; it has also been found that when using sodium nitrite, the reaction proceeds slowly and a large excess of nitrite and acid is needed in

30 order to obtain the iodine almost quantitatively in reasonable time. Also most of the other oxidizing agents do not come into consideration. Chlorine occasions formation of

35 iodic acid, from which the iodine cannot be obtained by adsorption in carbon. Experiments with iron chloride have showed that also here the separation takes place slowly, whereas the iron creates trouble, detrimental to the later adsorption. The solution filtered

40 after the treatment still gives a distinct colouring with carbon disulphide, which shows that the iodine had not yet been completely precipitated.

45 Experiments with potassium permanganate however have showed that with the the-

oretical quantity of this substance and exceedingly little acid a quantitative separation takes place practically immediately.

The invention consists in a process for liberating iodine from iodine-containing spring-waters, in which an exceedingly small quantity of acid and approximately the theoretical quantity of potassium permanganate is added to neutralized spring-water, after which the liberated iodine is adsorbed directly in charcoal or other adsorption agent. 55

The important advantages which are obtained with this invention may appear from the following comparative experiments.

(1) To 250 ccm. of neutral iodine-containing water (in which the iodine is present as sodium iodide) with a content of 39.6 mg. iodine per liter are added 65

0.5 ccm. normal sulphuric acid plus the theoretical quantity of sodium nitrite and 70  
10 ccm. carbon disulphide.

Within an hour the liberation of the iodine commences and increases slowly.

After 24 hours 40% of the iodine is separated. 75

After 48 hours 60% of the iodine is separated.

After 5 days it can be proved, after addition of a new quantity of carbon disulphide, that the iodine is completely separated. 80

(2) To 100 ccm. of a perfectly neutralized iodine-containing water, containing 10 mg. iodine as sodium iodide, 0.15 ccm. sodium nitrite (10% solution) and 0.2 ccm. normal sulphuric acid (theoretically 0.054 ccm. nitrite solution and 0.16 ccm. normal sulphuric acid would be sufficient) are added. 85

After 24 hours 6 mg. iodine or 60% is separated.

(3) To 100 ccm. iodine-containing water of the same composition as in experiment 2 are added 90

0.15 ccm. sodium nitrite and  
0.5 ccm. normal sulphuric acid. 95

After 1/2 hour 9 mg. iodine are now separated.

After 20 hours the complete separation of 10 mg. iodine is effected.

(4) To 100 ccm. iodine-containing water 100

of the same composition as in experiments 2 and 3 are added

0.15 ccm. sodium nitrite and

2.5 ccm. normal sulphuric acid.

5 The separation of the iodine now is instantaneous and complete.

(5) 100 ccm. iodine water as above is mixed with a solution of 2.5 mg. potassium permanganate and 0.2 ccm. normal sulphuric acid

10 (theoretically required 2.5 mg.  $KMnO_4$  and 0.13 ccm. normal  $H_2SO_4$ ). Here the

iodine is liberated immediately and quantitatively. Also with less sulphuric acid this result is still obtained. In the treatment of

15 1 million liters iodine water per day the 5th experiment requires, as compared to the third, a smaller consumption of sulphuric acid of 150 kg. per day, which in the Dutch

20 East Indies amounts to a saving of approximately \$10. Further 10% more iodine is obtained therewith, as it is technically impracticable to spend 20 hours on liberating the

25 iodine, during which time also a part of the iodine would doubtless be lost by evaporation.

The high cost of chemicals for the separation of iodine with sodium nitrite and sulphuric acid is just the reason why people in

30 Java have returned in many instances to the separation of iodine as cuprous iodide.

The present invention therefore effects an important saving in chemicals, as not only

35 much less sulphuric acid is necessary but also so much less permanganate that the cost

35 hereof is much less than the otherwise cheaper nitrite.

Furthermore the separation of the iodine takes place instantaneously and quantitatively, so that one can commence immediately

40 with the adsorbing of the liberated iodine by charcoal, without losing iodine by evaporation through long duration of the reaction, as can take place when the work is done with sulphuric acid and sodium nitrite

45 and when working without a great excess of these chemicals, which excess is not economical and therefore often avoided. This latter case causes in practice a considerably smaller

50 recovery of the iodine than the water originally contains.

In carrying out the process the procedure is preferably as follows:

Before separating the iodine, the iodine-containing water must be completely neutralized, the same as is the case with the nitrite method. To this end the bi-carbonates are

55 preferably converted into insoluble salts and separated according to any known suitable method. The water, which is now only

60 weakly alkaline, is then neutralized completely with sulphuric acid, for which only a little sulphuric acid is necessary. Then the

neutral iodine-containing water is acidified with very little sulphuric acid, namely to a

65 very weak acid reaction. Thereupon potas-

sium permanganate is added according to the invention, namely for every gram of iodine which the water contains, 0.25 g. potassium permanganate is added. Only a very weak acid reaction of the iodine water is necessary and the potassium permanganate is then reduced directly to manganous salt without formation of manganese dioxide. The solution remains clear; no colloidal metal hydroxide formation takes place, which otherwise could work unfavourably on the adsorption of the iodine by the charcoal. It is also disadvantageous to take an excess of potassium permanganate, on account of the cost, as because, after the liberation of the iodine any possible organic compounds present are oxidized, be it only slowly, by the superfluous potassium permanganate, with which a separation of manganese hydroxide could take place, which, as stated above, works disadvantageously on the adsorption power of the charcoal.

What I claim is:—

1. Process for extracting iodine from iodine-containing spring-waters, which comprises neutralizing the spring-water, mixing it with an exceedingly small quantity of acid and approximately the theoretical quantity of potassium permanganate and adsorbing the extracted iodine immediately afterwards.

2. Process for extracting iodine from iodine-containing spring-waters which comprises neutralizing the spring-water, mixing it with an exceedingly small quantity of acid and approximately the theoretical quantity of potassium permanganate and with an adsorbing agent.

3. Process for extracting iodine from iodine-containing spring-waters which comprises neutralizing the spring-water, mixing it with an exceedingly small quantity of acid and approximately the theoretical quantity of potassium permanganate and with charcoal.

FRITS ELLINGER.